

Feb. 13, 1940.

R. WARNECKE

2,189,971

SECONDARY ELECTRON EMITTING ELECTRODES

Filed Oct. 15, 1937



INVENTOR  
ROBERT WARNECKE

BY

*H.S. Brown*  
ATTORNEY

## UNITED STATES PATENT OFFICE

2,189,971

SECONDARY ELECTRON EMITTING  
ELECTRODE

Robert Warnecke, Paris, France, assignor to  
Compagnie Generale de Telegraphie Sans Fil,  
a corporation of France

Application October 15, 1937, Serial No. 169,172  
In France October 23, 1936

2 Claims. (Cl. 250—174)

This invention relates to secondary electron emitting electrodes suitable for use in so-called electron multipliers.

It is well known that most pure metals have rather slight secondary emission, and it is the usual practice in electron multipliers to increase the secondary electron emission by covering an ordinary metal electrode with a layer of substance of more intense emission. For example, 10 use has been made of a layer of a deposit of an alkali metal on an oxidised metal base, one typical case being where caesium, oxide of caesium and silver are used.

Known electrodes of this nature have, however, the disadvantage of exhibiting rather low thermal stability. Moreover, even when used in a fairly high vacuum, the active emitting surface coating is liable to damage or destruction by bombardment of positive ions. They are, 15 therefore, not very suitable for use in tubes which may have to dissipate high power and in other cases where the electrodes in question operate at rather high temperatures of the order of 800 to 1,000° C.

The present invention seeks to avoid these defects and limitations and provides electrodes having good power of secondary emission while able to resist large rises of temperature.

In accordance with the invention use is made 30 of a basis metal such as copper alloyed with a metal having low work function such as beryllium.

An electrode made of or covered with one of the above alloys is treated by heating in a high 35 vacuum so as to drive off occluded gases. This process imparts a physical structure which greatly improves its secondary electron emission power.

The proportion of beryllium to the copper can 40 be varied within fairly wide limits and may be from 1% to 10% by weight of the alloy.

The accompanying drawing shows curves connecting the secondary emission factor  $n$  (ratio of the number of secondary electrons emitted 45 per incident primary electron) with velocity  $v$  (abscissae) of primary electrons expressed in volts.

The curves 1, 2, 3, 4 and 5 were obtained with

an electrode of an alloy of copper and beryllium with 2.4% of beryllium; the curve 1 at ordinary temperature, the curve 2 at 700° C., the curve 3 at 800° C., and the curve 4 at 900° C. In each case the electrode was first thermally treated and degassed as above stated.

Curve 5 was obtained for the same conditions as curve 1 that is to say cold, but after 100 hours of operation.

Curve 6 is a curve for pure copper.

These curves show that the secondary electron emissivity or multiplication effect does not exhibit appreciable fatigue and is practically independent of temperature up to about 1,000°. The slight increase of the multiplication effect when 15 the temperature rises is probably attributable to the fact that the metal becomes gradually cleaner in proportion to the increase of temperature.

The thermal treatment of the alloy for which 20 curves 1, 2, 3, 4, 5 were obtained, was carried out as follows: the temperature was raised gradually (for about one hour) up to about 850° C. and then maintained at this temperature for about 2½ hours in a pressure below  $8.10^{-6}$  mm. of mercury (during the first hour), the final pressure being less than  $2.10^{-7}$  mm. of mercury.

The power of secondary emission obtained is a little below that of electrodes covered with certain complex substances, but, on the other hand 30 the electrodes of this invention are more easy to manufacture and of much better thermal stability which last renders them very useful in high power tubes.

What I claim is:

1. A secondary electron emitting electrode for 35 electron multipliers and the like having a surface composed of an alloy of which the secondary electron emissivity is several times that of copper and is substantially independent of temperature and which consists of from 1% to 10% of beryllium and the balance of copper.

2. A secondary electron emitting electrode for 40 electron multipliers and the like having a surface of high secondary electron emissivity and composed of a copper beryllium alloy consisting of 2½% beryllium and the balance copper.

ROBERT WARNECKE.